

## UNITED STATES PATENT OFFICE

2,145,756

## METALLIC BLAST MATERIAL

John F. Ervin, Ann Arbor, Mich.

No Drawing. Application September 11, 1936,  
Serial No. 100,386

3 Claims. (Cl. 51—280)

The invention relates to such metal abrasive materials as are used in the blast cleaning of iron, other castings, steel, stone, enamel-ware or other objects where the blast material is thrown by air or steam pressure or by mechanical force against them or used as an abrasive medium for sawing, cutting or polishing stone or other materials. Such metal abrasives are principally iron containing over 1% in carbon and .00% to 5% chromium and up to 5% nickel and up to 3.5% molybdenum and up to .5% vanadium.

Metal abrasives are now produced, that are principally iron with an approximate analysis of carbon 2.50%; manganese .50%; silicon 1.5%; sulphur .10%; phosphorus .40% balance mostly iron.

The life of an abrasive used in blasting is due to the resistance to breaking down under impact due to the high velocity of the abrasive when it strikes the object to be cleaned. The life is also governed by the resistance to wear or abrasion.

The power of resistance to failure by impact of a blast material is increased to a great extent by the addition of vanadium and chromium in the ratio of approximately 1 to 50, i. e. 1 part of vanadium to 50 parts of chromium.

The power of resistance to failure by crushing of a blast material to a definite degree of fineness is greatly increased by the addition of molybdenum and nickel in the ratio of 1 to 5; i. e. one part of molybdenum to 5 parts of nickel.

I claim:

1. An abrasive material comprising discrete particles of an alloy which is characterized by a high impact and abrasion resistance, such particles consisting of effective amounts and up to 5% of chromium; effective amounts and up to 5% of nickel; effective amounts and up to 1.0% of molybdenum; effective amounts and up to .1% of vanadium; substantially 1% of carbon, the

remainder of the alloy consisting of iron with small amounts of impurities, such as manganese, silicon and phosphorus, in insufficient quantity to alter the characteristics of the alloy; the alloy being further characterized in that the 5 vanadium content is adjusted to substantially one-fiftieth of the chromium content.

2. An abrasive material comprising discrete particles of an alloy which is characterized by a high impact and abrasion resistance, such particles consisting of effective amounts and up to 5% of chromium; effective amounts and up to 5% of nickel; effective amounts and up to 1.0% of molybdenum; effective amounts and up to .1% of vanadium; substantially 1% of carbon, the 15 remainder of the alloy consisting of iron with small amounts of impurities, such as manganese, silicon and phosphorus, in insufficient quantity to alter the characteristics of the alloy; the alloy being further characterized in that the 20 molybdenum content is adjusted to substantially one-fifth of the nickel content.

3. An abrasive material comprising discrete particles of an alloy which is characterized by a high impact and abrasion resistance, such particles consisting of effective amounts and up to 5% of chromium; effective amounts and up to 5% of nickel; effective amounts and up to 1.0% of molybdenum; effective amounts and up to .1% of vanadium; substantially 1% of carbon, the 25 remainder of the alloy consisting of iron with small amounts of impurities, such as manganese, silicon and phosphorus, in insufficient quantity to alter the characteristics of the alloy; the alloy being further characterized in that the 30 vanadium content is adjusted to substantially one-fiftieth of the chromium content and the molybdenum content is adjusted to substantially one-fifth of the nickel content.

JOHN F. ERVIN. 40